

# UNITED STATES PATENT OFFICE.

WILLIAM M. BURNHAM, OF CHICAGO, ILLINOIS.

## ANTI-FRICTION METAL.

SPECIFICATION forming part of Letters Patent No. 308,874, dated December 9, 1884.

Application filed January 31, 1884. (Specimens.)

*To all whom it may concern:*

Be it known that I, WILLIAM M. BURNHAM, residing at Chicago, in the county of Cook and State of Illinois, and a citizen of the 5 United States, have invented a new and useful Improvement in Anti-Friction Metal, of which the following is a full description.

It has been the common practice in the manufacture of anti-friction metals for journal-bearings and other analogous uses to combine plumbago with various metals in various proportions and by numerous methods; but in every instance as now practiced the plumbago has been mixed with the various metals 15 in such manner as to destroy the tenacity and toughness of the metal, thereby greatly reducing the wearing property of the composition, and consequently the value of the anti-friction metal for the purpose for which it is 20 used.

The object of this invention is to confine the plumbago in metals so as to have its particles held in their natural state without being mixed and permanently united with the 25 metals, leaving the plumbago free to separate and be set free as the metals by which it is confined wear away, and thereby prevent, to a large extent, the heating of the journal and its box, and decreasing the rapid wearing 30 from this cause; and this object I accomplish as hereinafter described.

The following metals, in the proportions named, will be found well adapted for wrapping up and holding the plumbago in its 35 natural state; but it is to be understood that any other combination of metals which, when fused or melted, will confine and retain the plumbago so that it can be readily set free can be used in place of the metals named. A mixture 40 of one hundred pounds is to be made up: of plumbago, ten pounds; copper, two pounds; antimony, five pounds; tin, ten pounds; brass, two pounds, and lead seventy-one pounds; but 45 these proportions can be varied to some extent so long as the variation does not prevent the

plumbago from being held in its natural and free state by the metals with which it is enveloped. The metals for the mixture are melted together, and when melted should be about the consistency of ordinary plasterer's mortar, so 50 as to be readily handled with a trowel, iron paddle, or any other suitable instrument by which it can be turned or brought into any desired shape, in much the same manner as soft putty or mortar can be handled, and when 55 in this state it is to be poured and wrapped over the plumbago without stirring or agitating, by which means the plumbago is enveloped by the metal, so that the particles are held in a natural state, being only confined 60 temporarily in the metal. This enveloping of the plumbago temporarily by the metal leaves it free, so as to separate from the metal part of the composition as the same wears away in use, allowing the plumbago to escape 65 in its natural state and come between the journal and the lining of the box and act to prevent any overheating of the parts. By thus enveloping or confining the plumbago temporarily with the metals the natural toughness 70 of the metals is not interfered with, and at the same time the grinding or rubbing of the anti-friction metal, as a whole, into fine powder by use is overcome, and the use of a lubricant is dispensed with, as the plumbago 75 acts and keeps the parts soft and pliable and in a clean, polished condition. The plumbago will be wrapped up, but held in cells formed around its particles.

What I claim as new, and desire to secure 80 by Letters Patent, is—

An anti-friction metal consisting of plumbago held in its natural state in a metallic envelope or cell without incorporation with metals, substantially as described.

WILLIAM M. BURNHAM.

Witnesses:

O. W. BOND,  
ALBERT H. ADAMS.